# EUROPEAN PATENT SPECIFICATION

(11) **EP 1 084 859 B1**
(45) Date of publication and mention of the grant of the patent: **10.11.2004**
(21) Application number: 99309175.0
(22) Date of filing: 18.11.1999
(51) Int. Cl.: B41M 5/00

(54) **Recording material**
Aufzeichnungsmaterial
Matériau d'enregistrement

(30) Priority: 17.09.1999 JP 26339699; 25.10.1999 JP 30241699
(43) Date of publication of application: 21.03.2001
(73) Proprietor: TEIKOKU PRINTING INKS MFG. CO., LTD, Tokyo 108 (JP)
(72) Inventor: Moriya, Kazuyoshi, Tokyo 116 (JP)
(74) Representative: Hallybone, Huw George

(56) References cited:
- EP-A- 0 701 179
- DATABASE WPI Section Ch, Week 199944 Derwent Publications Ltd., London, GB; Class A12, AN 1999-521971 XP002137808 & JP 11 227316 A (OJI PAPER CO), 24 August 1999 (1999-08-24)
- DATABASE WPI Section Ch, Week 199129 Derwent Publications Ltd., London, GB; Class F09, AN 1991-211666 XP002137893 & JP 03 133685 A (OJI PAPER CO), 6 June 1991 (1991-06-06)

## Description

### BACKGROUND OF THE INVENTION

### 1. Field of the Invention

The present invention relates to a recording material for use in recording by a visual recording method by means of printing, writing, or the like.

### 2. Description of the Related Art

Conventionally, in case of performing various existing recording such as printing on a plastic sheet, etc. by an oil-based ink, a water-based ink, and an UV curable ink, toner printing (a copy by a copy machine), thermal transfer printing, ink-jet printing, writing by a water-based pen, writing by an oil-based pen, writing by a pencil, stamp sealing, vermilion inkpad sealing or the like, it was difficult to perform all the records efficiently on a species of recording material, in particular a recording material in which a plastic sheet is a base material.

In consequence, a reception layer corresponding to a record method in each record method is provided on a surface such as the plastic sheet, and then each record is generally performed.

According to such the method, however, the record reception layer corresponding to the record method in each record method must be provided, and intricacy is apt to occur inevitably.

EP-A-0701179 discloses a printing plate comprising an image receiving layer provided on a surface of plastic film, wherein the image receiving layer comprises two kinds of extender pigments having different average particle size ranges to impart unevenness to surface of the image receiving layer.

JP-A-11227316 discloses a recording medium having an ink receiving layer containing two kinds of amorphous silica having different average particle sizes.

### SUMMARY OF THE INVENTION

Therefore, it is an object of the present invention to provide a recording material provided with a multifunctional record reception layer which is capable of coping with various species of record method as described.

Furthermore, it is another object of the present invention to provide a recording material in which, in the case where recording is performed with drawings, characters or the like by the aforesaid various existing record methods, the drawings or the characters are clearly recorded without smears and stains, and furthermore the recorded drawings or characters have excellent strength, for example excellent water-resistance, rub-resistance, or the like.

In order to resolve the aforesaid problems, the present invention provides a recording material in which a resin layer containing both of a large particle size sponge silica having a particle size 8 to 18µm and a small particle size sponge silica having a particle size 1 to 7µm is provided as a record reception layer on at least one face of a base material. The pore volume of said silica is 0.7 to 7 ml/g. The sponge silica is manufactured by a gelling method.

The base material used for the present invention is not in particular restricted if the base material is a material on which a record reception layer can be provided, but in a material in which the base material per se does not also contain a plurality of species of record reception property, effects of the present invention are especially great. As such the base materials, a film, a sheet, a plate, a spin-coated CD disc or the like composed of polyethylene, polypropylene, polyester, polycarbonate, polymetaacrylate, a metal or the like are illustrated. Furthermore, as the base material of the present invention, a paper, a synthetic paper or the like can also be illustrated.

It is preferable that a pore volume of the silica used for the present invention is 0.8 to 4ml/g. If the pore volume of silica is too small, there is a tendency that the record reception property of the reception layer is lowered. Furthermore, if the pore volume of silica is too large, the viscosity of the resin liquid substance constituting the reception layer is conspicuously high, and there is a tendency that a coat operation is conspicuously difficult in a manufacture of the recording material (according to another aspect of the present invention).

As the resin liquid substance, a resin solution, a resin emulsion, a melted hot melt resin, a two-part curing type uncured resin, an ultraviolet rays curing type uncured resin , or the like can be illustrated. As operations of curing after these resin agents are coated or printed on the base material, evaporation, cooling, or heating of a solvent or a dispersing medium, or ultraviolet rays irradiation or the like is adopted in response to each substance. According to the present invention, use of a non-water-soluble resin is preferable in order to attain excellent water-resistance.

The large particle size sponge silica and the small particle size sponge silica are both used in the record reception layer in the present invention. The large particle size silica has a particle size of 8 to 18µm. And if only the large particle size silica is used, there occurs drawbacks that sedimentation of silica occurs in the resin agent and it is easy to cause quality variations in the reception layer, and further rub-resistance of the reception layer is lowered, etc.

Furthermore, if only the small particle size silica of a particle size 1 to 7µm is used, a reduction in reception performance is caused, and objects of the present invention cannot be attained.

Furthermore, concerning a ratio of an amount of large particle size silica used to an amount of small particle size silica, it is preferable that a weight ration of the small particle size silica to the large particle size silica is about 0.1 to 5. By using at this ratio or so, it becomes easy to eliminate both drawbacks and maintain merits by synergism.

Furthermore, the record reception layer in the present invention contains silica and a resin. In the relationship of the silica amount and the resin amount, if the former is too much, a reduction in the rub-resistance of the record reception layer is caused, and if the latter is too much, a reduction in reception performance is caused. Accordingly, it is preferable that a resin of 15 to 150 pts.wt. per 100 pts.wt. of silica is used.

Furthermore, it is preferable that the pore volume of silica is about 0.8 to 4ml/g as described above. If the pore volume is too small, a reduction in the reception performance is caused, and there is a tendency that the rub-resistance is also lowered. If the pore volume rate is too large, it becomes easy to cause a reduction in strength such as the rub-resistance of the record reception layer. Furthermore, it is not necessarily necessary that the pore volumes of the large particle size silica and small particle size silica are the same.

Furthermore, in the reception layer of the present invention, in addition to silica and a binder resin, additives such as silica of a particle size 7 to 8 µm, a surfactant, a leveling agent, a dye fixing agent, various pigments, various fillers or the like can from time to time be used as an object demands.

Sponge silica which is a structural element according to the present invention will be described, and the sponge silica means silica of a sponge-like structure having many pores in silica particles. As a manufacture of silica, a sedimenting method and a gelling method exist, and it is possible to obtain silica which has a sufficient pore volume in case of using the gelling method. Thus, the sponge silica which is a structural element according to the present invention is manufactured by the gelling method.

Furthermore, the present invention provides the recording material in which the reception layer is provided on one face of the plastic sheet and the adhesives layer is provided on the other one face. This adhesives layer is freely peeled off and re-adhered, preferably. This adhesives layer which is freely peeled off is formed by applying or drying an adhesives solution or an emulsion containing an adhesive minute sphere of a particle size 2 to 100µm on the base material, or formed by applying a radioactive rays curing ink on the base material, and next irradiating radioactive rays.

As for an applying method, any one of screen printing, offset printing, photogravure printing, flexographic printing, letter press printing, roll coating, spray coating and the like may be used, and the screen printing in which a film thickness of the adhesive layer can be increased is the most suitable. A pattern of printing or coating when the adhesive layer is formed may be set solid all over, set linear, set dotty, or set designed, and the printing or coating may be performed in an area of 10% or more of a sheet-like base material, preferably 20% or more thereof. The film thickness of the adhesive layer is preferably 4µm or more, and it is particularly desirable that the film thickness is 10µ m or more from a viewpoint of re-exfoliation and adhesive stability.

### DESCRIPTION OF THE PREFERRED EMBODIMENT

After a coat agent composed of 50 pts.wt. of silica of a pore volume 1.9ml/g and a particle size 11µm, 50 pts.wt. of sponge silica of a pore volume 1.7ml/g and a particle size 5µm, and 500 pts.wt. of acrylate emulsion of resin concentration 10% is coated on a polyester sheet, water is heated and evaporated, to form a recording material A in which a reception layer is provided on one face of a polyester sheet. Furthermore, recording materials B, C, D, E, F, G are made according to the similar step. A composition of the reception layer of these recording material is designated on Table 1.

**(Table 1)**

| Recording Material | Silica of Large Particle Size | Silica of Small Particle Size | Resin |
|---|---|---|---|
| A | 50 pts.wt. of pore capacity 1.9ml/g and particle size 11µm | 50 pts.wt. of pore capacity 1.7ml/g and particle size 5µm | 50 pts.wt. of acrylate |
| B | 80 pts.wt. of the ditto silica | 20 pts.wt. of the ditto silica | 50 pts.wt. of the ditto resin |
| C | 20 pts.wt. of the ditto silica | 80 pts.wt. of the ditto silica | 50 pts.wt. of the ditto resin |
| D | 50 pts.wt. of the ditto silica | 50 pts.wt. of the ditto silica | 100 pts.wt. of the ditto resin |
| E | 50 pts.wt. of pore capacity 1.0ml/g and particle size 12µm | 50 pts.wt. of pore capacity 3.0ml/g and particle size 5µm | 50 pts.wt. of the ditto resin |
| F | - | 100 pts.wt. of pore capacity 1.7ml/g and particle size 5µm | 50 pts.wt. of the ditto resin |
| G | 50 pts.wt. of pore capacity 0.1ml/g or less and particle size 11µm of non-sponge silica | 50 pts.wt. of pore capacity 0.1ml/g or less and particle size 5µm of non-sponge silica | 50 pts.wt. of the ditto resin |

Next, the same characters and drawings are recorded on the reception layer face of these recording materials A to G by oil ink printing, toner printing (a copy by a copy machine), thermal transfer printing, ink-jet printing, recording by a water pen, recording by a pencil, stamp sealing, or vermilion inkpad sealing, and the resultants are shown in Table 2. As shown in Table 2, Embodiments 1 to 5 use each of the recording materials A to E shown in Table 1, and Comparative Examples 1, 2 use the recording materials F, G.

**(Table 2)**

| Embodiments and Comparative Examples | Recording Material | Recording Method and Evaluation | | |
|---|---|---|---|---|
| | | Oil Ink Printing | Toner Printing (a copy by a copy machine) | Thermal Transfer Printing |
| Embodiment 1 | A | ○ | ○ | ○ |
| Embodiment 2 | B | ○ | ○ | ○ |
| Embodiment 3 | C | ○ | ○ | ○ |
| Embodiment 4 | D | ○ | ○ | ○ |
| Embodiment 5 | E | ○ | ○ | ○ |
| Comparative Example 1 | F | ○ | ○ | × |
| Comparative Example 2 | G | ○ | ○ | × |

| | Recording Material | Recording Method and Evaluation | | |
|---|---|---|---|---|
| Embodiments and Comparative Examples | | Ink-Jet Printing | Water Pen Recording | Oil pen Recording |
| Embodiment 1 | A | ○ | ○ | ○ |
| Embodiment 2 | B | ○ | ○ | ○ |
| Embodiment 3 | C | ○ | ○ | ○ |
| Embodiment 4 | D | ○ | ○ | ○ |
| Embodiment 5 | E | ○ | ○ | ○ |
| Comparative Example 1 | F | × | × | ○ |
| Comparative Example 2 | G | × | × | ○ |

| | Recording Material | Recording Method and Evaluation | | |
|---|---|---|---|---|
| Embodiments and Comparative Examples | | Pencil Recording | Stamp Sealing | Vermilion Inkpad Sealing |
| Embodiment 1 | A | ○ | ○ | ○ |
| Embodiment 2 | B | ○ | ○ | ○ |
| Embodiment 3 | C | ○ | ○ | ○ |
| Embodiment 4 | D | ○ | ○ | ○ |
| Embodiment 5 | E | ○ | ○ | ○ |
| Comparative Example 1 | F | ○ | × | × |
| Comparative Example 2 | G | ○ | × | × |

However, mark ○ in Table 2 indicates that both definition and rub-resistance of records are excellent, and mark × indicates that one or both of them is inferior. Incidentally, in the definition of the records, the decision was made by visual observation. Furthermore, in the rub-resistance, the decision was made according to whether or not characters and drawings were blurred by rubbing the characters and drawings which were printed, written and sealed by a finger.

As can be seen from Table 2, the embodiments 1 to 5 were excellent in the definition and rub-resistance of records in any one of the various present record methods (the oil ink printing, the toner printing (a copy by a copy machine), the thermal transfer printing, the ink-jet printing, the entering by a water pen, the entering by an oil pen, the entering by a pencil, the stamp sealing, and the vermilion inkpad sealing).

Incidentally, the adhesives layer or the adhesives layer which can be freely peeled off is provided on a back face of the sheet of these embodiments 1 to 5, so that the sheet which is excellent in the definition and the rub-resistance of the records and can be held to a glass face, a desk face, or the like by the adhesives layer can be attained.

As described above, according to the present invention, in the case where recording is performed with drawings, characters or the like by the various present record methods, the drawings or characters are clearly recorded without being ink-stained, and furthermore it is possible to provide the recording material in which the recorded drawings or characters display excellent strength, for example excellent rub-resistance, or the like. Furthermore, it is possible to also provide the recording material which is excellent in the vivid record and rub-resistance, and can be adhered or re-exfoliated.

## Claims

1. A recording material, wherein a resin layer which contains both of a large particle size sponge silica having a particle size 8 to 18 µm and a small particle size sponge silica having a particle size 1 to 7 µm is provided as a record reception layer on at least one face of a base material, **characterised in that** the pore volume of the large particle size sponge silica and small particle size sponge silica is 0.7 to 7 ml/g and that the silica particles are manufactured by a gelling method.

2. A recording material according to claim 1, wherein a weight ratio of the small particle size silica to the large particle size silica is 0.1 to 5.

3. A recording material according to claim 1 or 2, wherein a pore volume of the large particle size silica and small particle size silica is 0.8 to 4 ml/g.

4. A recording material according to claim 1, 2, or 3, wherein the resin layer contains 15 to 150 pts.wt. of a resin per 100 pts.wt. of all weight of silica.

5. A recording material according to any one of claims 1 to 4, wherein the base material is a plastic sheet.

6. A recording material according to claim 5, wherein the record reception layer is provided on one face of the plastic sheet and an adhesives layer is provided on the other face.

7. A recording material according to claim 6, wherein the adhesives layer is made of adhesives which can freely be peeled off and stick again.

8. A method of manufacturing a recording material according to any one of claims 1 to 5, wherein after a liquid substance in which silica is scattered in a resin liquid substance is coated or printed on the base material, a resin is cured.

## Patentansprüche

1. Aufzeichnungsmaterial, wobei eine Harzschicht, die sowohl ein schwammartiges Siliziumdioxid mit einer großen Teilchengröße, das eine Teilchengröße von 8 bis 18 µm aufweist, als auch ein schwammartiges Siliziumdioxid mit einer kleinen Teilchengröße, das eine Teilchengröße von 1 bis 7 µm aufweist, enthält, als eine Aufzeichnungsempfangsschicht auf mindestens einer Seite eines Basismaterials bereitgestellt ist, **dadurch gekennzeichnet, daß** das Porenvolumen des schwammartigen Siliziumdioxids mit großer Teilchengröße und des schwammartigen Siliziumdioxids mit kleiner Teilchengröße 0,7 bis 7 ml/g beträgt, und daß Siliziumdioxidteilchen durch ein Gelverfahren hergestellt sind.

2. Aufzeichnungsmaterial nach Anspruch 1, wobei ein Gewichtsverhältnis des Siliziumdioxids mit kleiner Teilchengröße zu dem Siliziumdioxid mit großer Teilchengröße 0,1 bis 5 beträgt.

3. Aufzeichnungsmaterial nach Anspruch 1 oder 2, wobei ein Porenvolumen des Siliziumdioxids mit großer Teilchengröße und des Siliziumdioxids mit kleiner Teilchengröße 0,8 bis 4 ml/g beträgt.

4. Aufzeichnungsmaterial nach Anspruch 1, 2 oder 3, wobei die Harzschicht 15 bis 150 Gew.-Teile eines Harzes, bezogen auf 100 Gew.-Teile des Gesamtgewichts an Siliziumdioxid, enthält.

5. Aufzeichnungsmaterial nach einem der Ansprüche 1 bis 4, wobei das Basismaterial ein Kunststoffblatt ist.

6. Aufzeichnungsmaterial nach Anspruch 5, wobei die Aufzeichnungsempfangsschicht auf einer Seite des Kunststoffblatts und eine Haftschicht auf der anderen Seite bereitgestellt ist.

7. Aufzeichnungsmaterial nach Anspruch 6, wobei die Haftschicht aus Haftmitteln hergestellt ist, die frei abgezogen werden kann und erneut kleben kann.

8. Verfahren zur Herstellung eines Aufzeichnungsmaterials nach einem der Ansprüche 1 bis 5, wobei, nachdem eine flüssige Substanz, in der Siliziumdioxid in einer flüssigen Harzsubstanz verteilt ist, auf dem Basismaterial beschichtet oder bedruckt ist, ein Harz gehärtet wird.

## Revendications

1. Matériau d'enregistrement, dans lequel une couche de résine contenant à la fois une silice poreuse de grosse granulométrie ayant une taille de particules de 8 à 18 µm et une silice poreuse de petite granulométrie ayant une taille de particules de 1 à 7 µm, est prévue pour servir de couche réceptrice d'enregistrement sur une face au moins d'un matériau de base, et **caractérisé en ce que** le volume des pores de la silice poreuse de grosse granulométrie et de la silice poreuse de petite granulométrie est de 0,7 à 7 ml/g et **en ce que** les particules de silice sont fabriquées par un procédé de gélification.

2. Matériau d'enregistrement selon la revendication 1, dans lequel le rapport en poids de la silice de petite granulométrie sur la silice de grosse granulométrie est de 0,1 à 5.

3. Matériau d'enregistrement selon la revendication 1 ou 2, dans lequel le volume des pores de la silice de grosse granulométrie et de la silice de petite granulométrie est de 0,8 à 4 ml/g.

4. Matériau d'enregistrement selon la revendication 1, 2 ou 3, dans lequel la couche de résine contient 15 à 150 parties en poids de résine pour 100 parties en poids du poids total de silice.

5. Matériau d'enregistrement selon l'une quelconque des revendications 1 à 4, dans lequel le matériau de base est une feuille plastique.

6. Matériau d'enregistrement selon la revendication 5, dans lequel la couche réceptrice d'enregistrement est prévue sur une face de la feuille plastique et une couche adhésive est prévue sur l'autre face.

7. Matériau d'enregistrement selon la revendication 6, dans lequel la couche adhésive est constituée d'adhésifs pouvant être décollés à recollés à volonté.

8. Procédé de fabrication d'un matériau d'enregistrement selon l'une quelconque des revendications 1 à 5, dans lequel la résine est durcie après qu'une substance liquide contenant de la silice répartie dans une substance liquide de résine ait été appliquée par enduction ou impression sur le matériau de base.
